

## UNITED STATES PATENT OFFICE

2,208,981

## STENCIL SHEET

Shinjiro Horii, Kanda-ku, Tokyo, Japan

No Drawing. Application June 21, 1939, Serial  
No. 280,381. In Japan May 16, 1939

2 Claims. (Cl. 41—38.6)

This invention relates to improvements in stencil sheets for use in duplicating manuscript or typewritten documents, drawings and the like and particularly stencil sheets of the type consisting of a sheet of fibrous material provided with a normally impervious coating in which characters may be formed by the pressure of a hand stylus or by the impact of the type of a writing machine.

10 The present invention is based upon the discovery that the mixture obtained by the incorporation of soybean casein with synthetic resins, emulsified and softened by emulsifiers and tempering agents or softening agents and dispersed into water or other dispersing medium, constitutes a highly efficient coating for stencil sheets, possessing flexibility and durability.

15 The soybean casein is specially prepared by extracting soybean with a solvent, such, for example, as a mixed solvent comprising methyl or ethyl alcohol and benzine or benzol, and drying out the solvent at low temperature. The temperature of the extraction and the drying must be kept as low as possible, avoiding the deterioration of the protein material.

20 Synthetic resins suitable for use with the protein material may be prepared by, for example, the condensation of aldehydes with phenols or amines, by the reaction of acid anhydrides with polyhydric alcohols and by the polymerization of unsaturated hydrocarbons or vinyl compounds. These polymerizable compounds may be incorporated with certain modifying agents before they are polymerized, thereby producing a suitably modified resin produced in accordance with the modifying agents incorporated with.

25 In carrying out the invention, the coating material is prepared by emulsifying and softening

the mixture of soybean casein with synthetic resins by the aid of emulsifying agents, such as soaps, Turkey-red oil, sulphate salts of the higher fatty alcohols, triethanolamine, lecithins or the like, and tempering agents, such as ethylene glycol, glycerine, sorbitol, fatty oils, fats, waxes, heavy mineral oils, naphthenic acid esters or a mixture containing two or more of these, and dispersing the mixture into water or other suitable dispersing medium, such as alcohols, solvent naphtha, cyclohexanol, butyl acetate, ethyl ethers of glycol or the like. Then the prepared coating material may be coated or impregnated with the fibrous base, such as Japanese Yoshino paper, in the usual manner.

30 The proportions of the ingredients of the coating material may vary according to several circumstances. The following is an example:

|                   | Parts by weight |     |
|-------------------|-----------------|-----|
| Soybean casein    | 20              | 20  |
| Phenolic resin    |                 | 5   |
| Triethanolamine   |                 | 5   |
| Turkey-red oil    |                 | 10  |
| Castor oil        |                 | 20  |
| Heavy mineral oil | 10              | 25  |
| Cyclohexanol      |                 | 20  |
| Water             |                 | 200 |

35 What I claim is:

1. A stencil sheet consisting of a base of fibrous material coated with a coating material including soybean casein, a synthetic resin, an emulsifying agent and a tempering agent.

2. A stencil sheet consisting of a base of fibrous material coated with a coating material including soybean casein, a phenolic resin, an emulsifying agent and a tempering agent.

SHINJIRO HORII.